

Aug. 16, 1932.

A. ELMENDORF

1,871,447

METHOD OF FLATTENING FLEXIBLE SHEETS FACED WITH WOOD

Filed May 16, 1931

Fig. 1.



Fig. 2.



Fig. 3.



Fig. 4.



Fig. 5.



Inventor:

Armin Elmendorf,

By W. F. Brandenrich,  
Attorney.

## UNITED STATES PATENT OFFICE

ARMIN ELMENDORF, OF CHICAGO, ILLINOIS, ASSIGNOR TO THE FLEXWOOD COMPANY,  
A CORPORATION OF DELAWARE

## METHOD OF FLATTENING FLEXIBLE SHEETS FACED WITH WOOD

Application filed May 16, 1931. Serial No. 537,803.

While the principal shrinkage of wood is across the grain, there is some shrinkage in the direction of the grain as the wood dries from the green state. This shrinkage in the lengthwise direction is not always uniform throughout a given piece of wood; the result being that, in the case of thin veneers, the unequal shrinkage lengthwise of the grain often produces what are known as "cockles", namely, bulges in areas where there has been less shrinkage than in the surrounding wood. Therefore, after drying, veneers in which this unbalanced longitudinal shrinkage occurs will not present smooth, flat surfaces; this being true even though the wood be disrupted along the lines of the grain to divide it into numerous closely spaced connected filaments; nor will the bulges or "cockles" be prevented by gluing the veneer to a flexible backing. This characteristic of veneer is not objectionable when the veneer can be glued to a rigid supporting surface under pressure, but it is highly objectionable in the case of thin veneers glued to paper, fabric, or other flexible backings and adapted to be cemented or pasted upon a wall or other surface without the employment of means to produce and maintain for a considerable time a pressure that will flatten out the veneer; the result being that, when the composite sheet, composed of the veneer and its flexible backing is pasted to a wall or other supporting surface, even though it be rolled flat to reduce the "cockles", the latter will immediately form again and pull the backing loose from the supporting surface, so that the composite sheet will appear to have blisters therein. This objectionable characteristic of wood veneer is encountered to such an extent that, in the commercial manufacture of flexible composite sheets composed of thin veneers and paper or fabric backings, as much as 20% of commercial veneers of some woods that are obtained for the manufacture of this product must be discarded. Thus, there is not only the waste of veneer, but the loss of time in inspecting each lot of veneers and culling out those sheets that are not satisfactory.

The object of the present invention is to make it possible, in a simple and inexpensive manner, to avoid the aforementioned objectionable consequences resulting from the tendency of some thin veneers to form surface irregularities or "cockles" due to unequal shrinkage in the direction of the grain, whereby flexible composite sheets, each composed of wood veneer and a backing, may safely be made of veneer subject to "cockles", without danger that the sheets will fail to remain flat after having been pasted or cemented to a wall or other surface.

I have found that, if thin, dry "cockled" veneer is flattened out and moderately heated, the pressure and the heat being maintained for a short time, the "cockles" will disappear; this being particularly true in the case of veneer glued to a flexible backing. If a composite flexible sheet, of which one element is a piece of veneer which has been thus treated, is pasted to a wall, for example, it will remain flat and will not thereafter present the appearance of containing blisters. Therefore, in the manufacture of flexible veneer-faced wall coverings, or the like, composed of wood veneer backed with paper, cloth, or other suitable flexible material, I first produce the composite sheet in the usual way, and then treat the composite sheet to remove the "cockles" in the veneer, pressing it between hot plates, causing the temperature of the sheet to be raised to about the boiling point of water, and maintaining the temperature and pressure until the desired results are secured; this requiring only a short period of time which ordinarily will be anywhere from one minute to ten minutes. When the composite sheets are treated in this manner, the need for culling out those sheets of veneer in which "cockles" are formed is obviated, and, since the cost of the additional treatment is much less than the waste resulting from the discarding of a considerable percentage of the veneers, flexible composite sheets, one face of which is wood veneer, may be manufactured more cheaply than heretofore.

The various features of novelty whereby my invention is characterized will herein-after be pointed out with particularity in the claims; but, for a full understanding of my

invention and of its objects and advantages, reference may be had to the following detailed description taken in connection with the accompanying drawing, wherein:

- 5 Figure 1 is a section through a flexible sheet composed of wood veneer and a backing cemented thereto, showing an irregularity due to unequal shrinkage of the veneer in the direction of the grain, the thicknesses being 70  
 10 greatly exaggerated; Fig. 2 is a section on line 2—2 of Fig. 1; Fig. 3 is a section taken at right angles to the plane of a composite sheet positioned between two hot plates, the thicknesses of the elements making up the 75  
 15 composite sheet being greatly exaggerated; Fig. 4 is a perspective view of a fragment of a panel that has been treated, illustrating the flatness of the surface; and Fig. 5 is a more or less diagrammatic view, illustrating a sheet 80  
 20 being passed between a roller and a concave steam chest in the manner of a piece of laundry going through an ironing machine.

Referring to Figs. 1 and 2 of the drawing, 1 represents a sheet of thin wood veneer 25 glued to a flexible backing 2 of cloth, paper or other suitable material. The thicknesses are greatly exaggerated in the drawing, as the veneer will ordinarily have a thickness of from  $\frac{1}{16}$  of an inch to  $\frac{1}{4}$  of an inch, although it may sometimes be somewhat thicker than this. Assuming that the grain runs parallel with the plane of the section on which Fig. 1 is taken and at right angles to the plane on which Fig. 2 is taken, unequal shrinkage of the veneer lengthwise of the grain often produces little raised areas or bulges, as indicated at 3. It will be seen that, if these bulges are not reduced, a sheet 30 containing them, when pasted on a wall in the manner of wall paper, will appear to have blisters. Even though the bulges or "cockles" be rolled flat, they will form again, pulling the backing away from the wall.

These bulges or "cockles" can be flattened 45 out, and, if the veneer be heated while they are in a flattened condition, the fiber or wood structure will take a set and afterwards remain flat. The degree of pressure employed is not important, except that it should be 50 sufficient completely to flatten out the bulges. Also, if the pressure be too great, the wood may have a polished and compressed appearance that may be undesirable. I have found that ordinarily a pressure of about fifty 55 pounds per square inch gives satisfactory results. There are limits to the temperature to which the wood, or rather the composite sheet, may be brought. If the temperature be too low, there will not be the permanent setting of 60 the reduced bulges in a flat state. If the temperature is too high, there will be, first, a deterioration of the glue joint, and, second, damage to the wood. I have found that a 65 temperature in the neighborhood of the boiling point of water gives the best results.

Of course, the temperature may be somewhat lower or appreciably higher. The time during which the work is subject to heat and pressure varies with different woods and different thicknesses of veneers. Sometimes the treatment may be completed in about a minute, whereas at other times it may take ten minutes.

One manner of applying the heat and pressure is illustrated in Fig. 3 in which there 75 are upper and lower hot plates A and B between which the composite sheet is laid. If desired, the composite sheet may be slowly passed through a rotary ironing machine, as indicated in Fig. 5, wherein X represents the sheet, C represents a stationary curved steam chest, and D represents a slowly rotating roller. One end of the sheet is inserted between the chest and the roller, so that the sheet is gradually drawn through 80 the machine, each portion thereof remaining under pressure between the chest and the roller for a sufficient length of time to effect 85 the intended result.

After the sheet has been treated in the 90 manner illustrated in Fig. 3 and Fig. 5, it has the appearance of a fragment shown in Fig. 4, the surface thereof being entirely flat.

The heating of the veneer softens the same 95 so that the structure thereof readjusts itself, the longer fibres that produced the bulges probably being compacted and thus shortened so as to have no longer any tendency to bow out of the plane of the sheet.

When speaking of veneer being "dry", I 100 mean veneer which in commerce is known as "dry veneer". In other words, my process is in no sense one whose purpose is to reduce the moisture content of wood as are ordinary drying processes, but one which 105 operates on a composite product, the veneer element of which has been dried previously.

I claim:

1. The method of eliminating bulges in 110 dry, thin wood veneer due to unequal shrinkage in the direction of the grain in drying from a green state, which consists in pressing the veneer flat, heating the veneer to a temperature in the neighborhood of the boiling point of water, and maintaining the pressure and the heat until the wood has softened.

2. The method of flattening a flexible composite sheet composed of a flexible backing 115 glued to thin wood veneer having therein bulges due to unequal shrinkage in the direction of the grain in drying from a green state, which consists in pressing the sheet flat, heating it to a temperature in the neighborhood of the boiling point of water, and maintaining the pressure and the heat until the wood has softened.

3. The method of insuring flatness of surface in a composite sheet composed of thin 120

70

75

80

85

90

95

100

105

110

115

120

125

130

wood veneer glued to a flexible backing and ruptured along the grain into many connected filaments, where the wood is of a type in which bulges result from uneven shrinkage in the direction of the grain in drying from a green state, which consists in pressing the sheet flat to reduce the bulges and heating it sufficiently to soften the wood while held flat.

10 4. The method of insuring flatness of surface in a composite sheet composed of thin wood veneer glued to a flexible backing and ruptured along the grain into many connected filaments, where the wood is of a type in which bulges result from uneven shrinkage in the direction of the grain in drying from a green state, which consists in pressing the sheet flat with sufficient force to flatten out the bulges and heating it to a 15 temperature in the neighborhood of the boiling point of water and maintaining the heat and pressure until the wood has softened.

20 In testimony whereof, I sign this specification.

25 ARMIN ELMENDORF.

30

35

40

45

50

55

60

65